# EUROPEAN PATENT SPECIFICATION

(11) **EP 2 109 544 B1**
(45) Date of publication and mention of the grant of the patent: **30.09.2020**
(21) Application number: 08709308.4
(22) Date of filing: 05.02.2008
(51) Int. Cl.: B41M 5/52, D21H 21/16, D21H 17/28, D21H 17/34, D21H 17/45

(54) **A METHOD FOR MAKING PRINTING PAPER AND A MIXTURE COMPOSITION**
VERFAHREN ZUR HERSTELLUNG VON DRUCKPAPIER UND GEMISCHZUSAMMENSETZUNG
PROCÉDÉ DE FABRICATION DE PAPIER D'IMPRESSION ET D'UNE COMPOSITION D'UN MÉLANGE

(30) Priority: 05.02.2007 FI 20070102
(43) Date of publication of application: 21.10.2009
(73) Proprietor: UPM-Kymmene Oyj, 00100 Helsinki (FI)
(72) Inventor: PYKÄLÄINEN, Nina, FI-53300 Lappeenranta (FI); VARVEMAA, Päivi, FI-53100 Lappeenranta (FI)
(74) Representative: Papula Oy
(86) International application number: PCT/FI2008/050040
(87) International publication number: WO 2008/110661

(56) References cited:
- EP-A1- 0 327 215
- EP-A1- 0 580 405
- EP-A2- 0 747 235
- EP-B1- 0 046 416
- WO-A1-98/32920
- WO-A1-99/54541
- WO-A1-2006/067273
- US-A- 5 672 392
- US-A1- 2002 046 820
- US-A1- 2005 032 642
- US-A1- 2005 032 642
- US-A1- 2005 107 254
- US-B1- 6 764 726

## Description

### FIELD OF THE INVENTION

The invention relates to a method for making printing paper as defined in the preamble of claim 1 and to a mixture composition for the surface-sizing of printing paper as defined in the preamble of claim 4.

### BACKGROUND OF THE INVENTION

Known from the prior art are various methods for making different kinds of printing papers. Also known from the prior art are different kinds of papers for use in printing, e.g. different types of inkjet-based printing.

As to the inkjet-based printing techniques, it is important to ensure sufficient printing ink absorption in the high speed inkjet papers to provide a sufficiently good colour print. The important criterion is that the printing inks of different colours do not blend together. In uncoated papers, sufficient absorption can be ensured by low hydrophobic sizing level of the base paper, which has been disclosed e.g. in patent application WO 2006067273.

It is known that anionic aqueous printing ink must be bound to the paper in order for the print to be waterfast. Waterfastness is essential for example in bank balance statements and other similar prints. It is known that waterfastness can be improved by adding cationic polymers to the surface-size or coating on the surface of the paper. The most commonly used polymer is polyDADMAC. Many of the fixatives used at the wet end of the paper machine are suitable for this purpose. Patent application WO 2006067273 discloses the surface treatment of printing paper with a cationic polymer together with an internal sizing treatment of the paper. The suggested optimal amount is 2g/m², in which case about half of the amount of the surface-size should be replaced with the cationic polymer. The amount of the cationic polymer as presented above increases the production costs of the printing paper.

From WO 98/32920, EP 0327215, US 5672392 and EP 0747235 are known different sizing or coating compositions and methods for surface sizing or coating of substrate. From US 6764726 is known an ink jet recording sheet having improved image waterfastness.

### OBJECTIVE OF THE INVENTION

The objective of the invention is to eliminate the drawbacks referred to above. One specific objective of the invention is to disclose a new method and surface-size mixture composition for making printing paper. In particular, the objective of the invention is to disclose a new way of improving printability of printing paper.

### SUMMARY OF THE INVENTION

The method and the mixture composition in accordance with the invention are characterized by what has been presented in the claims.

The invention is based on a method for making printing paper, which method comprises forming an uncoated paper. In accordance with the invention, a surface-size mixture comprising starch and polyvinyl pyrrolidone and cross-linker is arranged on the surface of the uncoated paper for improving printability of the paper, and the surface-size mixture comprises 45 - 99% starch, 1 - 50% polyvinyl pyrrolidone and less than 5 % cross-linker which is epoxy-based or glycosal-based cross-linker, and the starch is cationic starch.

Printability means print quality, waterfastness and/or degree and rate of absorption. Print quality means print sharpness and/or evenness.

The invention is specifically based on improving inkjet printability in uncoated papers by a new surface-size composition.

In this context, paper means any fibre-based paper, board or fibre product or the like. The paper may have been made from chemical pulp, mechanical pulp, chemimechanical pulp and/or the like. The paper may be in the form of a wet web, dried web or sheet, or in other form which is suitable for the purpose. The paper may comprise suitable fillers and additives.

In one embodiment of the invention, uncoated fine paper which mainly does not comprise mechanical pulp, e.g. WFU or UWF, is used in the method. Alternatively, it is possible to use uncoated paper which does comprise mechanical pulp, e.g. SC paper or newsprint.

One embodiment of the invention comprises producing high speed inkjet paper with good printability.

In one embodiment of the invention, the surface-size mixture is in the form of a solution, dispersion or paste. The mixture can be arranged or applied on the surface of the paper by any manner known per se in the art.

In one embodiment, the surface-size mixture is arranged on the surface of the formed paper web in conjunction with the web formation, e.g. in conjunction with the drying. In one embodiment, the mixture is arranged on the surface of the formed web in a separate step after the formation of the web.

In one embodiment of the method, a base paper web is formed in a manner known per se and cut to the correct width. The web is coated with the surface-size mixture. If desired, the web is cut into sheets or the like, and the web or the paper products cut off from it are provided with the desired print in the desired manner. In one embodiment, the print can be provided by a digital printing method, e.g. inkjet-based technique.

Furthermore, the invention is based on a mixture composition to be used for making printing paper. In accordance with the invention, the mixture composition comprises starch and polyvinyl pyrrolidone and cross-linker and the mixture composition comprises 45 - 99% starch, 1 - 50% polyvinyl pyrrolidone and less than 5 % cross-linker which is epoxy-based or glycosal-based cross-linker, and the starch is cationic starch, and the mixture composition can be arranged on the surface of an uncoated paper as surface-size.

The mixture composition comprises less than 5% cross-linker. The cross-linker may be e.g. an epoxy-based, a glycosal-based or a zirconium-based cross-linker.

In one embodiment of the invention, the mixture composition comprises a cationic polymer. In one embodiment, the mixture composition comprises less than 15% cationic polymer.

The mixture composition comprises 45 - 99% starch.

The mixture composition comprises 1 - 50% polyvinyl pyrrolidone. The polyvinyl pyrrolidone may be in any state and be present as a pure agent or mixture.

The method and the surface-size mixture in accordance with the invention provide considerable advantages compared to the prior art.

The surface-sizing composition in accordance with the invention provides a printing paper of excellent print quality and improved printability characteristics. Furthermore, the surface-sizing composition in accordance with the invention provides quicker colour absorption / setting rate in the printing.

The invention provides an industrially applicable, easy and fast way of making printing paper. The method in accordance with the invention is easy, simple and affordable to be executed as a production process.

The method in accordance with the invention is suitable to be used for making different kinds of printing papers, specifically for making inkjet-type, such as high speed inkjet, printing papers.

### DETAILED DESCRIPTION OF THE INVENTION

### Example 1

The tests of this example involved examining different kinds of surface-sizing compositions to be used in WFU paper for high speed inkjet printing. The tests were conducted in a laboratory scale.

The tests involved examining and testing the effect of PVP (polyvinyl pyrrolidone) as a surface-sizing agent in non-pigmented compositions for surface-sizing of paper. The obtained results were compared to the results obtained with a reference composition. The reference composition used comprised mainly a starch-containing surface-size mixture without any PVP content.

The base paper used in the tests was a low internal-sized uncoated fine paper with the basis weight of about 82g/m² and Cobb values of about 60 - 70g/m². The paper was surface-sized on one side with an RK laboratory coater and a rod at about 3g/m². The surface-size mixture compositions are presented in Tables 1 and 2. The pH value of the surface-size mixture was 7.5.

The surface-sized papers were printed by two inkjet printers; Epson Stylus C46 with Versamark ink and Canon Pixma iP3000.

The printed papers were rated as to the printing ink absorbency, line spreading and roughness, waterfastness (K,M), wet rub and densities. The visual properties of the printed papers were examined by three persons.

Waterfastness means blackness after wetting / blackness before wetting x 100%. A higher value indicates better waterfastness; the value may exceed 100%. Wet rub means blackness of the white area after rubbing / blackness of the black area before rubbing. A lower value indicates better wet rub x 100%; the value may be zero.

Table 1 presents the agents used in the tests. Table 2 presents the surface-sizing agent compositions used in the individual tests. The solids content of the compositions was about 12%. Table 3 presents the results analysed from the printed paper.

**Table 1**

| Agent | Agent composition |
|---|---|
| A | cationic starch |
| B | PVP (polyvinyl pyrrolidone) aqueous solution |
| C | cationic polyalkylamide polymer |
| D | epoxy-based cross-linker |
| E | glycosal-based cross-linker |

In the tests, the N-vinyl-2-pyrrolidone homopolymer was used as the PVP. It dissolves in water and many organic solvents, such as alcohols, amines, acids, chlorinated hydrocarbons and amides. In a solution, it exhibits excellent wetting properties and good film-forming capability. It is more hydrophilic than starch and a better OBA activator, but it is more difficultly cross-linked.

**Table 2**

| Composition | Ref | 8 | 9 | 15 | 20 |
|---|---|---|---|---|---|
| A | 100 | 70 | 50 | 90 | 70 |
| B | | 30 | 50 | 10 | 30 |
| C | 15 | 15 | 15 | 15 | 15 |
| D | | | | | 5 |
| E | 5 | 5 | 5 | 5 | |

**Table 3**

| Rating, lower value = better result | Ref | Test 8 | Test 9 | Test 15 | Test 20 |
|---|---|---|---|---|---|
| Absorption | 1 | 1 | 1 | 1,5 | 2 |
| Waterfastness | 1-2 | 1-2 | 2 | 0,5 | 0,5 |
| Wet rub | 2 | 1 | 2 | 0,5 | 1 |
| Print mottling, Griffin | 2-3 | 1 | 1 | 1,5 | 2 |
| Density (K) | 3 | 2 | 2 | 2 | 1 |
| Density (C) | 3 | 3 | 2 | 2 | 1,5 |

The tests showed that the use of PVP together with starch in the surface-sizing provided good waterfastness and wet rub to the printed paper, substantially without reducing the density compared to other compositions. PVP was found to remain on the surface of the paper, i.e. it exhibits lower migration into paper than starch. Faster ink absorption, lower ink spreading and better waterfastness were therefore obtained with the PVP. Fast ink absorption rate is useful because it reduces the spreading of the ink.

The tests showed that PVP together with starch improves considerably the waterfastness of the print and the black and white print quality, such as print sharpness and evenness, compared to the paper treated with the reference mixture (Ref).

In summary of the tests one can conclude that PVP together with starch provides a very effective composition for surface-sizing of printing paper.

### Example 2

The tests of this example involved examining different surface-sizing compositions to be used in WFU paper for high speed inkjet printing. The tests were conducted in a pilot scale.

The tests involved examining and testing the effect of PVP (polyvinyl pyrrolidone) as a surface-sizing agent in non-pigmented compositions for surface-sizing of paper. The obtained results were compared to the results obtained with a reference composition. The reference composition used comprised mainly a starch-containing surface-size mixture without any PVP content.

The base paper according to Example 1 was used in the tests, and it was coated accordingly with a surface-size mixture at 2.5g/m². The surface-size mixture compositions are presented in Table 4. The solids content of the compositions was 12%.

The papers were printed by inkjet printers; Epson Stylus C48 with Versamark ink, Canon Pixma iP3000 and HP Deskjet 6540.

**Table 4**

| Composition | Ref | 5 | 6 | 7 | 8 | 11 |
|---|---|---|---|---|---|---|
| A | 100 | 70 | 70 | 70 | 90 | 50 |
| B | | 30 | 30 | 30 | 10 | 50 |
| SMA, Impress SC 740 | | | | 5 | | |
| C | 15 | 15 | 15 | 15 | 15 | 15 |
| D | 5 | | 5 | 5 | | |
| E | | 5 | | | 5 | 5 |

In the tests, it was found that the Digat absorption time was reduced when using PVP in the surface-size composition, compared to the results obtained with the reference surface-size mixture. In the tests, the absorption time for black ink when using PVP (compositions 5-8 and 11) was in the range of 100 - 200ms, and when using only starch (Ref) it was more than 300ms.

Waterfastness was found to be good in all compositions, preferably more than 100%. Also wet rub was good in all compositions, preferably less than 12%.

Also colour density was found to be at a good level when using PVP, irrespective of the printing device, relative to the results obtained with the reference composition.

### Example 3

This test involved examining printing of papers that were surface-sized with the compositions in accordance with Test 2 by digital high speed inkjet printing machines.

Waterfastness, wet rub, waterbleed, colour density, print evenness and print-through were found to be good with all compositions containing PVP relative to the reference composition.

Waterbleed means blackness of the white area after wetting / blackness of the black area before wetting x 100%. A lower value indicates better result. The goal is a result of less than 10%; the value may be zero.

Furthermore, it was found in the tests that the setting time of Digat ink was shorter when using a PVP-containing surface-size composition compared to the reference composition. The setting time with the PVP-containing composition was mainly less than 150ms.

Runnability and printability of the paper which contains PVP in the surface-sizing composition were found to be good in the printing tests.

In the printing tests of Examples 2 and 3, composition 8 with 10 parts PVP and 90 parts starch seemed to emerge as the preferred surface-sizing mixture composition.

Results from the pilot tests (Example 2) and printing tests (Example 3) supported the results obtained in the laboratory scale. A PVP-containing surface-size composition provides an excellent printing paper with good printability and print quality.

The method in accordance with the invention is suitable in different embodiments to be used for making the most different kinds of printing papers.

The invention is not limited merely to the examples referred to above; instead many variations are possible within the scope of the inventive idea defined by the claims.

## Claims

1. A method for making printing paper, which method comprises forming an uncoated paper, **characterized in that** a surface-size mixture containing starch and polyvinyl pyrrolidone and cross-linker is arranged on the surface of the uncoated paper for improving printability of the paper, and the surface-size mixture comprises 45 - 99% starch, 1 - 50% polyvinyl pyrrolidone and less than 5 % cross-linker which is epoxy-based or glycosal-based cross-linker, and the starch is cationic starch.

2. The method in accordance with claim 1, **characterized in that** the surface-size mixture is in the form of a solution or dispersion.

3. The method in accordance with claim 1 or 2, **characterized in that** a high speed inkjet paper with good printability is produced

4. A mixture composition to be used for making printing paper, **characterized in that** the mixture composition comprises starch and polyvinyl pyrrolidone and cross-linker and the mixture composition comprises 45 - 99% starch, 1 - 50% polyvinyl pyrrolidone and less than 5 % cross-linker which is epoxy-based or glycosal-based cross-linker, and the starch is cationic starch, and the mixture composition is arranged as a surface-size on the surface of an uncoated paper.

5. The mixture composition in accordance with claim 4, **characterized in that** the mixture comprises a cationic polymer.

## Patentansprüche

1. Verfahren zur Herstellung von Druckpapier, wobei das Verfahren das Ausbilden einen unbeschichteten Papiers umfasst, **dadurch gekennzeichnet, dass** eine Flächengrößenmischung (surface-size mixture), die Stärke und Polyvinylpyrrolidon und Vernetzer enthält, auf der Oberfläche des unbeschichteten Papiers aufgetragen wird und so die Bedruckbarkeit des Papiers verbessert wird, und dass die Flächengrößenmischung 45 - 99% Stärke, 1 - 50% Polyvinylpyrrolidon und weniger als 5% Vernetzer, welcher ein Vernetzer auf Epoxidbasis oder Glykosalbasis ist, umfasst, und dass die Stärke kationische Stärke ist.

2. Verfahren gemäß Anspruch 1, **dadurch gekennzeichnet, dass** die Flächengrößenmischung in der Form einer Lösung oder Dispersion vorliegt.

3. Verfahren gemäß Anspruch 1 oder 2, **dadurch gekennzeichnet, dass** ein Hochgeschwindigkeitstintenstrahlpapier mit guter Bedruckbarkeit hergestellt wird.

4. Mischungszusammensetzung zur Verwendung bei der Herstellung von Druckpapier, **dadurch gekennzeichnet, dass** die Mischungszusammensetzung Stärke und Polyvinylpyrrolidon und Vernetzer umfasst und dass die Mischungszusammensetzung 45 - 99% Stärke, 1 - 50% Polyvinylpyrrolidon und weniger als 5% Vernetzer, welcher ein Vernetzer auf Epoxidbasis oder Glykosalbasis ist, umfasst, und dass die Stärke kationische Stärke ist, und dass die Mischungszusammensetzung als eine Flächengröße auf der Oberfläche eines unbeschichteten Papiers ausgebildet ist.

5. Mischungszusammensetzung gemäß Anspruch 4, **dadurch gekennzeichnet, dass** die Mischung ein kationisches Polymer umfasst.

## Revendications

1. Procédé pour fabriquer du papier d'impression, lequel procédé comprend la formation d'un papier non couché, **caractérisé en ce qu'**un mélange d'encollage en surface contenant de l'amidon et de la polyvinylpyrrolidone et un agent de réticulation est disposé sur la surface du papier non couché pour améliorer l'imprimabilité du papier, et le mélange d'encollage en surface comprend 45 à 99% d'amidon, 1 à 50% de polyvinylpyrrolidone et moins de 5% d'agent de réticulation qui est un agent de réticulation à base d'époxy ou à base de glycosal, et l'amidon est l'amidon cationique.

2. Procédé selon la revendication 1, **caractérisé en ce que** le mélange d'encollage en surface se présente sous forme d'une solution ou d'une dispersion.

3. Procédé selon la revendication 1 ou 2, **caractérisé en ce que** du papier pour jet d'encre à vitesse élevée ayant une bonne imprimabilité est produit.

4. Composition de mélange à utiliser pour la fabrication de papier d'impression, **caractérisée en ce que** la composition de mélange comprend de l'amidon et de la polyvinylpyrrolidone et un agent de réticulation et la composition de mélange comprend 45 à 99% d'amidon, 1 à 50% de polyvinylpyrrolidone et moins de 5% d'agent de réticulation qui est un agent de réticulation à base d'époxy ou à base de glycosal, et l'amidon est l'amidon cationique, et la composition de mélange est disposée comme encollage en surface sur la surface d'un papier non couché.

5. Composition de mélange selon la revendication 4, **caractérisée en ce que** le mélange comprend un polymère cationique.
